

# UNITED STATES PATENT OFFICE.

ALFRED J. LIEBMANN, OF NEW YORK, N. Y.

## COMPOSITION OF MATTER AND PROCESS OF MAKING THE SAME.

1,177,119.

Specification of Letters Patent. Patented Mar. 28, 1916.

No Drawing.

Application filed March 12, 1915. Serial No. 13,936.

To all whom it may concern:

Be it known that I, ALFRED J. LIEBMANN, a citizen of Switzerland, residing at No. 55 West Ninety-fifth street, in the city, county, 5 and State of New York, have invented certain new and useful Improvements in Compositions of Matter and Processes of Making the Same; and I do hereby declare the following to be a true and exact description 10 thereof.

The object of my invention is to provide a new composition of matter which may be used for many useful purposes, as for electrodes and brushes for dynamos and electric 15 motors.

I have found that the metal tungsten when properly mixed with carbon or copper or both of them, produces a composition of matter which has great advantages for use 20 in the electrical art, for the purposes above stated. Such a composition of matter is of excellent wearing quality and its use as a brush for electric machinery eliminates to a great degree the objectionable sparking and 25 other troubles.

The modern art of producing tungsten metal has been so far developed that it is possible to obtain tungsten metal either in the form of very fine and soft black powder 30 or in the form of coarse, hard and grainy powder or in any of the intermediate forms.

I have discovered that the best brushes will be obtained by a mixture of carbon and tungsten; or of carbon, copper and tungsten.

35 A great advantage arising from my composition is that it can be made with any proportions of material suited for the special purpose for which it is desired. If the material is to be used as a brush in a slow moving machine, less hardness is required, while if it is to be used for a brush in a fast moving machine, a harder material is required. The degrees of hardness of my composition of matter are regulated by the degrees of hardness 40 and the proportions of the tungsten used. The finer the tungsten powder, the softer it is, and the softer the composition of which it is a constituent. On the other hand, the coarser the grain of the tungsten 45 powder, the harder it is, and the more hardness it gives to the composition of material of which it is a constituent. In a machine which generates low currents, more tungsten could be used than in one which generates 50 very high currents, because the conductivity 55 of tungsten is not as high as copper and in

the case of high currents, I have found it advisable to counter-balance this property of tungsten by an increased admixture of copper. As mentioned above, a very wide 60 range for the manufacture of my invention is given by the innumerable different grades of hardness and size of grain which can be obtained of tungsten and the different proportions of its admixture. These qualities 65 of tungsten allow a brush to be made of almost any hardness and with a very wide range of electrical conductivity.

In the carrying out of my invention, while it is possible to simply take the carbon or graphite powder and mix it with tungsten powder, or tungsten and copper powder together and compress the mixture under a high pressure and then heat it in a vacuum, 70 or an inert atmosphere to obtain a solid 75 cake of the mixture, I have found it to be of great advantage to follow a more specific procedure.

I have obtained the very best results in 80 mixing the carbon or graphite powder and powdered tungsten with an amalgam of copper, such amalgam containing about two parts of mercury to one part of copper, and then grinding together the carbon, the amalgam and the tungsten powder into a uniform mass in a mortar or similar device. This ground mass is then placed into a mold 85 of the shape desired for the brush or the electrode and exposed to a very high pressure, by hydraulic or other means, of about twenty to forty tons per sq. inch. Under 90 this pressure, the mercury is almost completely pressed out of the cracks of the mold and can be collected in its pure state and used over again. The remaining cake is then 95 slowly heated to a temperature of about 300 degrees to 400 degrees C. which heating may be done in the open air. I have, however, found it preferable to first heat the cake below red heat in air and then to carry out 100 and continue the heating process in vacuum or in an inert atmosphere, to prevent oxidation and to facilitate the driving off of the last traces of mercury remaining after the compression.

105 After the heating, the cake consists of a solid piece of a mixture of either carbon and tungsten, copper and tungsten or carbon tungsten and copper and is at once ready to be used as an electrode or as a brush in an electric machine.

110 Any desired hardness may be obtained by

varying the amounts of tungsten, copper or mercury and by varying also the pressure applied when the mixture is being molded.

Instead of using an amalgam, I have found that I can use most any other material of binding qualities which can be volatilized without leaving any foreign traces in the perfected cake or composition. I can also use many organic binders which carbonize, thereby changing slightly the percentage of the carbon in the finished products. A very good inorganic binder is cadmium-bismuth-amalgam, but I have found that even water alone can be used with good success. As organic binders, I have found very useful alcohol, glycerin, sugar-syrups, gum-tragacanth solution, starch solution, collodium and others. When using the cadmium-bismuth-amalgam mixed with copper, carbon and tungsten or carbon and tungsten alone, after the pressing operation, the mercury as well as the bismuth and cadmium are volatilized by heat in hydrogen or in an inert atmosphere or in vacuum.

When using the organic binders above mentioned, or an inorganic binder such as water, these binders can be completely volatilized after the compression, leaving the carbon, copper and tungsten product or the carbon and tungsten product depending upon the material used in the mixture.

The cakes comprising my improved composition of matter are molded into shapes for use as electrodes, or as brushes in electric machinery or whatever form desired as above described.

Having now described my invention, what I claim as new and desire to secure by Letters Patent, is:—

1. A composition of matter consisting of a mixture of carbon, copper and tungsten.
2. A composition of matter consisting of a compressed body composed of a mixture of powdered carbon, powdered copper and powdered tungsten.
3. A composition of matter consisting of a compressed body of powdered carbon and tungsten.
4. An electric contact consisting of a mixture containing powdered tungsten.
5. An electric contact consisting of a compressed mixture containing powdered tungsten.
6. An electric contact consisting of a compressed mixture of carbon, copper and tungsten.

7. The process consisting of mixing carbon, copper amalgam and tungsten, subjecting the mixture to a high pressure and volatilizing the remaining mercury.

8. The process consisting of mixing a binder with carbon, copper and tungsten, subjecting the mixture to a high pressure, and volatilizing the binder.

In witness whereof I have hereunto set my hand at the borough of Manhattan, city and State of New York, this tenth day of March, 1915.

ALFRED J. LIEBMANN.  
In presence of—

ETHEL D. BARON,  
JOHN J. RANAGAN.